

July 19, 1938.

E. VAN DER PYL

2,124,279

ABRASIVE WHEEL

Filed Oct. 9, 1936



FIG. 3

FIG. 2

FIG. 6



FIG. 5

Inventor

FIG. 4

EDWARD VAN DER PYL

By George Geomert  
Attorney

## UNITED STATES PATENT OFFICE

2,124,279

## ABRASIVE WHEEL

Edward Van der Pyl, Holden, Mass., assignor to  
Norton Company, Worcester, Mass., a corpora-  
tion of Massachusetts

Application October 9, 1936, Serial No. 104,860

5 Claims. (Cl. 51—209)

The invention relates to abrasive wheels and also other abrasive bodies and with regard to its more specific features to a grinding disk for grinding on the flat face thereof.

5 One object of the invention is to provide a method for the manufacture of an abrasive article as above characterized which is relatively inexpensive and according to which manufacture of a wheel can be quickly accomplished. Another 10 object of the invention is to provide an inexpensive and satisfactory bond for abrasive bodies. Another object of the invention is to provide an efficient cold setting bond. Other objects will be in part obvious or in part pointed out hereinafter.

The invention accordingly consists in the features of construction, combinations of elements and arrangements of parts, and in the several steps and relation and order of each of said steps 20 to one or more of the others thereof, all as will be illustratively described herein, and the scope of the application of which will be indicated in the following claims.

In the accompanying drawing illustrating one 25 of many possible embodiments of the mechanical features of this invention,

Figure 1 is a plan view of a mounting plate and wire reinforcement upon which the abrasive disk may be formed.

30 Figure 2 is an enlarged fragmentary cross sectional view, taken on the line 2—2 of Figure 1.

Figure 3 is a perspective view of a nut.

Figure 4 is a sectional view of a mold illustrating a preferred manner of manufacturing the 35 abrasive article.

Figure 5 is a fragmentary sectional view of part of the mold after the pressing operation,

Figure 6 is a side elevation of the completed disk and mounting.

40 Referring first to Figures 1 and 4, I provide a mounting or backing plate in the form of a steel disk 10 having a central axial hole 11, a plurality of countersunk holes 12 close to the hole 11, and a plurality of additional countersunk holes 13 distributed over the plate 10. Referring now to

45 Figure 2, in each hole 13 is located a screw 14. I provide, as shown in Figures 1, 2, and 4, a steel wire mesh 15 cut to annular shape. I place the wire mesh 15 upon the plate 10 with the screws 50 14 projecting through openings. I then fasten the parts together by means of nuts 16, the nuts being formed so that they will interlock with the meshes as clearly shown.

The foregoing constitutes a backing plate to 55 which is firmly united the screen mesh 15. I now

mold a grinding disk in situ upon the backing plate and around the screen mesh in the following manner.

I provide abrasive grain of any desired abrasive material, for example fused alumina or silicon carbide, emery or corundum, or diamonds. I prefer to use fused alumina and silicon carbide. I provide a quantity of cast iron in finely divided form, for example iron filings which will pass through a 30 mesh screen or finer. I provide a 10 quantity of sal ammoniac. The proportions of the ingredients may be widely varied but for purposes of illustration satisfactory results may be achieved using 40 parts of abrasive grain, 40 parts of iron filings, and two to ten parts of sal 15 ammoniac, all by weight. I mix these ingredients thoroughly in any suitable manner and add enough water to wet the mixture thoroughly.

Referring now to Figure 4, I mount the plate 10 upon the bottom plate 20 of a mold. An annular mold ring 21 of a diameter the same as the diameter of the plate 10 is now placed around the plate 10, as shown in Figure 4, suitable spacers 22 being used if desired. I next place upon the plate 10 a central plug core 23 having a central 25 pin 24 which fits in the hole 11.

I now fill the space between the core 23 and the ring 21 with the desired quantity of the mixture made as hereinbefore specified. I then place a top plate 25 upon the abrasive mixture. The 30 entire mold is then pressed between the platten 26 and the top plate 27 of a suitable press. I may press to definite volumetric limits and the pressing is preferably of the order of several thousand pounds to the square inch in order thoroughly to 35 compact the mass.

Sal ammoniac, otherwise known as ammonium chloride ( $\text{NH}_4\text{Cl}$ ) together with water and iron forms a solution at room temperatures in which some of the iron becomes  $\text{FeCl}_3$  and some of it 40 precipitates as iron hydroxide. The iron chloride is a satisfactory bond even though mixed with some iron hydroxide and a satisfactory reaction takes place during and after a cold pressing operation. The bond sets complete in a few hours 45 after the wheel is pressed.

The bond is relatively soft and therefore a grinding disk of free cutting characteristics is produced. I may use diamonds as the abrasive and form a wheel or an annulus thereof with or 50 without the special structural features described and illustrated. Diamonds bonded with the bond herein described are found to be effective for the grinding of tungsten carbide and similar materials.

It will thus be seen that there has been provided by this invention an article and a method in which the various objects hereinbefore set forth together with many thoroughly practical advantages are successfully achieved. As various possible embodiments might be made of the mechanical features of the above invention and as the art herein described might be varied in various parts, all without departing from the scope of the invention, it is to be understood that all matter hereinbefore set forth or shown in the accompanying drawing is to be interpreted as illustrative and not in a limiting sense.

I claim:—

15 1. An abrasive article comprising abrasive grain and a bond mainly comprising iron and ferric chloride.

2. An abrasive article comprising abrasive grain and a bond which is the reaction product of iron filings and sal ammoniac.

3. An abrasive product comprising abrasive grains and a bond resulting from the reaction of iron with a halide of ammonia.

4. The method of making an abrasive article which consists in providing a quantity of abrasive grain, mixing the abrasive grain with comminuted iron, a halide of ammonia and water, pressing and allowing to set cold.

5. An abrasive article comprising abrasive grain and a bond comprising ferric chloride, iron hydroxide and iron in an intimate mixture.

15

EDWARD VAN DER PYL.